# EUROPEAN PATENT SPECIFICATION

(11) **EP 0 018 152 B1**
(45) Date of publication and mention of the grant of the patent: **14.09.1983**
(21) Application number: 80301113.9
(22) Date of filing: 08.04.1980
(51) Int. Cl.: G21F 9/00, B24C 1/00

(54) **Decontamination method**
Entseuchungsverfahren
Procédé de décontamination

(30) Priority: 12.04.1979 US 29598
(43) Date of publication of application: 29.10.1980
(73) Proprietor: WESTINGHOUSE ELECTRIC CORPORATION, Pittsburgh Pennsylvania 15222 (US)
(72) Inventor: Marchese, Robert Thomas, Murrysville Pennsylvania (US)
(74) Representative: van Berlyn, Ronald Gilbert

## Description

This invention relates to decontamination methods and more particularly to methods for decontaminating components of nuclear power plants.

During the operation of nuclear power plants and similar apparatus, certain components become exposed to radiation and may develop a thin radioactive film on the surface of the component. From time to time, it is necessary to either inspect or repair these components of the nuclear reactor power plant. During the inspection or repair of the components, it is necessary for working personnel to enter the component or to be stationed in close proximity to the component whereby working personnel may be exposed to radiation emitted from the contaminated component. In some circumstances, the radiation field emitted from these components is such that a worker would receive the maximum permissible radiation dose in less than five minutes of working time. Such a situation means that a given worker may only spend a relatively short amount of time working on the inspection or the repair operation of the nuclear component. Having each worker spend a relatively short amount of time in the repair or inspection procedure, necessitates the use of many workers with each worker working a short time period in order to accomplish the desired procedure. While this may be an acceptable practice for minor inspections or repair procedures, this is not an acceptable practice where there is an extensive inspection or an extensive repair job to be performed. Where the procedure to be performed is a time consuming procedure, it is likely that an unusually large number of highly trained personnel would be necessary to carry out the task. Such a situation may not only be unacceptable from a financial aspect, but may also be unacceptable from a man-power level aspect. From Eur. 4186 d, Europaische Atomgemeinschaft-Euratom, Mosselmans G. and Nienhaus J., "Auswahl von Abrasiven und Badzusatzen fur die Dekontaminierung mittels Schlammstrahlen," 1968, a method of decontaminating components, especially components of nuclear power plants, is known. According to that document, the components are exposed to a jet of a sludge to remove the radioactive particles therefrom and, at the same time, to wash the radioactive particles away from said components without damaging the metal surface of the component.

It is the principal object of the present invention to provide a similar decontamination method with which radioactive particles are safely and rapidly washed away from contaminated components without damage to the components and to such a complete degree that working personnel may perform operations without fear of radiation exposure.

With this object in view, the present invention resides in a method of decontaminating metal components, especially components of nuclear power plants, wherein the components are exposed to a jet of a water-grit mixture to remove radioactive particles therefrom and, at the same time, to wash the radioactive particles away from said components without damaging the metal surface of the component, characterized in that said jet of water-grit mixture has a grit concentration of from 3% to 7% by weight and is emitted from a nozzle which is moved along said components at a distance of 15 cm to 25 cm from the surface of said component with an angle of impingement of between 30° to 70° and at a speed of 30 cm/min to 90 cm/min for intense particle removing action.

The flow rate and pressure of the water jet are controlled so that a thin layer of metal oxide deposits may be removed from the components without damaging the metal components thereby greatly reducing the radioactivity of the components. The grit types, size, and concentration in the water jet are also controlled along with the distance of the nozzle from the surface of the component and the angle of impingement so that an optimum level of decontamination is achieved without deterioration of the metal surface.

The invention will become more apparent from the following description of a preferred embodiment thereof shown, by way of example only, in the accompanying drawing, wherein the single figure is a diagram of apparatus used to perform the decontamination method.

During operation of typical nuclear power plants, certain components of the nuclear power plant such as the nuclear steam generators, become radioactively contaminated. Since certain repair or inspection operations that must be performed periodically on the nuclear power plant components require working personnel to be present in or near the components, it is important that the radiation field associated with the component be at a level that is compatible with the presence of working personnel for an extended period of time. The invention, described herein, is a method for decontaminating components of nuclear power plants so that working personnel may perform operations thereon.

Referring to the drawing, apparatus for performing the decontamination method comprises a platform 10 for supporting container 12 which may be a steel drum having a closure plate 14. Container 12 comprises supports 16 for supporting the specimen 18 to be decontaminated. Container 12 also has a vent 20 and a drain 22. Container 12 is arranged such that the front portion thereof is supported by a bar 24 so that container 12 is tilted such that liquid within container 12 will flow through drain 22. Drain 22 is connected to filter 26 which may be a 5-25,um filter bag chosen from those well known in the art. Filter 26 is connected to a pipe 28 which is connected to a drain for disposing of or recirculating the water used in the decontamination process. A 2.3 cm diameter tube 30 extends through universal joint 32 and closure plate 14 so that the front end of tube 30 is disposed within container 12. A nozzle 34 is mounted on the front end of tube 30 and is also connected to flexible hose 36. Nozzle 34 may be chosen from those well known in the art such as a "Dynajector" manufactured by the Aqua-Dyne Engineering, Inc. of Houston, Texas. Flexible hose 36 extends through closure plate 14 and is connected to grit supply 38 for supplying grit to nozzle 34. Tube 30 is connected to pump 40 which may be a 40 horsepower pump which is also connected to water supply 42 for supplying water to nozzle 34. Nozzle 34 provides a mechanism for mixing the grit and water and for emitting the water-grit mixture from nozzle 34 toward specimen 18. Tube 30 is also attached to drive mechanism 44 which may be a mechanism for controlling the horizontal movement of tube 30 and nozzle 34. Drive mechanism 44 may be chosen from those well known in the art.

The decontamination method comprises introducing water through tube 30 at a pressure between 140 x 10⁵ Pa (140 kg/cm²) and 190 x 10⁵ Pa (190 kg-cm2). The water flow rate at this pressure should be approximately 30 to 34 litres per minute through nozzle 34. Several types of grit may be used for mixing with the water such as alumina or magnetite. However, the grit size should be approximately 120 (about 125,um sieve opening) to 325 (44,urn sieve opening) mesh size in accordance with United States Sieve Series Mesh Sizes. It is important to note that the grit concentration in the water spray should be approximately 3% to approximately 7% by weight. In order to provide effective decontamination without excessive metal deterioration, it is important that the nozzle be placed approximately 15 cm to 25 cm from the surface of specimen 18. It has also been found that nozzle 34 should be arranged so that the water-grit mixture impinges the surface of specimen 18 at approximately between a 30°-70° angle and preferably at about 45°.

### Operation

In operation, a test specimen 18 having top surface that has been contaminated with radioactivity is placed within container 12 and supported by supports 16 as shown in the drawing. Closure plate 14 is then attached to container 12 such that tube 30, nozzle 34, and flexible hose 36 are arranged as shown in the drawing. Universal joint 32 which also comprises a clamping mechanism is arranged such that the flow of the water-grit mixture from nozzle 34 is directed to the proper elevation of specimen 18. At this point, nozzle 34 is approximately 15 to 25 cm from the surface of the specimen 18. Next, pump 40 is activated which causes water to be pumped from water supply 42 through tube 30 and into nozzle 34. The flow of water through nozzle 34 creates a vacuum in nozzle 34 which draws the grit from grit supply 38 through flexible hose 36 where it mixes with the water in nozzle 34. The water-grit mixture is then directed toward the specimen 18. Simultaneously, drive mechanism 44 is activated which causes tube 30 and nozzle 34 to move in a horizontal line across specimen 18 at a speed of approximately 30 cm per minute to approximately 90 cm per minute. The speed of travel of nozzle 34 is correlated with the water-grit flow rate so as to provide effective decontamination without excessive deterioration of the metal of specimen 18. The water and grit mixture impinges on the surface of specimen 18 and removes a thin oxide layer from the specimen which is carried away by the water-grit mixture and drains through drain 22 into filter 26. Once nozzle 34 has made a complete horizontal pass of specimen 18, universal joint 32 is readjusted so that nozzle 34 is directed toward a different vertical elevation of specimen 18 and at the same 15 to 25 cm distance. Then, drive mechanism 44 is reversed so that nozzle 34 makes a similar horizontal pass of speciment 18 but at a different elevation. In this manner, an entire sweeping of specimen 18 may be made. In addition to the apparatus as shown in the drawing, an additional nozzle 34 may be attached to tube 30 and also arranged at approximately a 45° angle and opposing the first nozzle 34 so as to provide a dual nozzle arrangement.

A test of the decontamination method was made with the following parameters:

Two passes were made across the surface of the specimen, one pass each at opposing 45° angles. This ensured cleaning of both sides of the irregularities in the surface of the specimen. Results of the tests show that 98.3% to 99.9% of the radioactive contamination was removed from the sample simulating nuclear reactor component surfaces. None of the samples suffered perceptible surface damage.

Tests and analysis have determined that with the use of the decontamination process, it is likely that less than 0.025 mm of metal surface will be removed from the specimen. It appears that the use of an alumina grit on Inconel metal will remove a metal layer of less than 0.0051-0.0076 mm and that the use of a magnetite grit on stainless steel will remove a metal layer of less than 0.012-0.025 mm.

While the decontamination method has been described as being used in a test apparatus, the decontamination method may be used on nuclear reactor components such as nuclear steam generators with the equipment adapted to be placed within the nuclear component. Therefore, the invention provides a decontamination method for lowering the radiation field of nuclear reactor power components so that working personnel may enter the component and perform operations thereon.

## Claims

1. A method of decontaminating metal components, especially components of nuclear power plants, wherein the components are exposed to a jet of a water-grit mixture to remove radioactive particles therefrom and, at the same time, to wash the radioactive particles away from said components without damaging the metal surface of the component, characterized in that said jet of water-grit mixture has a grit concentration of from 3% to 7% by weight and is emitted from a nozzle (34) which is moved along said components at a distance of 15 cm to 25 cm from the surface of said component (18) with an angle of impingement of between 30° and 70° and at a speed of 30 cm/min to 90 cm/min for intense particle removing action.

2. A method as claimed in claim 1, characterized in that said mixture is discharged with an angle of impingement of approximately 45° relative to the surface of said components.

3. A method as claimed in claim 1 or 2, characterized in that said grits have a size of between 120 mesh (about 125,um sieve opening) and 325 mesh (44_{1L}m sieve opening).

4. A method as claimed in any of claims 1 to 3, characterized in that said water-grit mixture is emitted at a pressure of between 140 x 10⁵ Pa (140 kg/cm²) to 190 x 10⁵ Pa (190 kg-cM²) and at a rate of between 30 and 34 liter/min per nozzle.

5. A method as claimed in any of claims 1 to 4, characterized in that said grit is alumina.

6. A method as claimed in any of claims 1 to 4, characterized in that said grit is magnetite.

## Revendications

1. Procédé pour décontaminer des éléments métalliques, en particulier des éléments de centrales électriques nucléaires, suivant lequel les éléments sont exposés à un jet d'un mélange d'eau et de matière abrasive pour enlever des particules radio-actives de ces éléments et en même temps éliminer par lavage les particules radio-actives de ces éléments sans détériorer leure surface métallique, caractérisé en ce que le jet de mélange d'eau et de matière abrasive a une concentration en matière abrasive de 3 à 7% en poids et est debité par une lance (34) qui est déplacée le long des éléments à une distance de 15 cm à 25 cm de la surface de l'élément (18) sous un angle d'impact compris entre 30 et 70° et à une vitesse de 30 cm/minute à 90 cm/minute pour une action intense d'élimination de particules.

2. Procédé suivant la revendication 1, caractérisé en ce que le mélange est débité sous un angle d'impact d'environ 45° par rapport à la surface des éléments.

3. Procédé suivant la revendication 1 ou 2, caractérisé en ce que les matières abrasives comportent des particules d'une granulométrie comprise entre 120 mesh (mailles d'environ 125 µm) et 125 mesh (mailles de 44 µm).

4. Procédé suivant l'une quelconque des revendications 1 à 3, caractérisé en ce que le mélange d'eau et de matière abrasive est projeté sous une pression comprise entre 140 x 10⁵ Pa (140 kg/cm²) et 190 x 10⁵ Pa (190 kg/cm2) et à un débit d'environ 30 à 34 litres/minute par lance.

5. Procédé suivant l'une quelconque des revendications 1 à 4, caractérisé en ce que la matière abrasive est de l'alumine.

6. Procédé suivant l'une quelconque des revendications 1 à 4, caractérisé en ce que la matière abrasive est de la magnétite.

## Patentansprüche

1. Verfahren für die Dekontamination von Bauteilen, insbesonder von Bauteilen von Kernkraftanlagen, bei dem die Teile einem Strahl von Wasser-Schmiergelteilchen-Mischung ausgesetzt werden, um radioaktive Teilchen davon zu entfernen und zur gleichen Zeit die radioaktiven ' Teilchen von den Bauteilen zu beschädigen, dadurch gekennzeichnet, das der Wasserstrahl von der Wasser-Schmiergelteilchen-Mischung einem Schmiergelteilchengehalt von 3 bis 7 Gew.% hat, und von einer Düse (34) abgegeben wird, die dem Bauteil (18) entlang mit einer Geschwindigkeit von 30 bis 90cm/min, mit einem Abstand von 15 bis 25 cm von der Oberfläche des Bauteiles (18) und mit einem Aufprallwinkel von 30 bis 70° auf die Bauteiloberfläche geführt wird, womit eine wirkungsvolle Entfernung radioaktiver Teilchen erreicht wird.

2. Verfahren nach Anspruch 1, dadurch gekennzeichnet, dass die Mischung mit einem Aufprallwinkel von etwa 45° auf die Bauteiloberfläche gerichtet wird.

3. Verfahren nach Anspruch 1 oder 2, dadurch gekennzeichnet, dass Schmiergelteilchen einer Grösse entsprechend 125 bis 44 micron Sieböffnung verwendet werden.

4. Verfahren nach einem der Ansprüche 1 bis 3, dadurch gekennzeichnet, dass die Wasser-Schmiergelteilchen Mischung unter einem Druck von 140 bis 190 kg/cm² und in einer Menge von etwa 30 bis 34 Vmin pro Düse abgegeben wird.

5. Verfahren nach einem der Ansprüche 1 bis 4 dadurch gekennzeichnet, dass die Schmiergelteilchen aus Aluminiumoxyd bestehen.

6. Verfahren nach einem der Ansprüche 1 bis 4, dadurch gekennzeichnet, dass die Schmiergelteilchen aus Eisenoxyd bestehen.
